

# United States Patent [19]

Horn et al.

[11] 4,326,895

[45] Apr. 27, 1982

[54] **PROCESS FOR MANUFACTURING ALUMINUM STRIP OR SHEET HAVING IMPROVED WELDABILITY**

[75] Inventors: Werner Horn, Singen; Jürgen Hennings, Gottmadingen, both of Fed. Rep. of Germany

[73] Assignee: Swiss Aluminium Ltd., Chippis, Switzerland

[21] Appl. No.: 141,430

[22] Filed: Apr. 18, 1980

[30] **Foreign Application Priority Data**

May 2, 1979 [DE] Fed. Rep. of Germany ..... 2917627

[51] Int. Cl.<sup>3</sup> ..... C22F 1/04

[52] U.S. Cl. ..... 148/11.5 A; 156/665;  
228/173 C

[58] **Field of Search** ..... 148/11.5 A; 156/629,  
156/645, 665; 228/173 C, 173 D

[56] **References Cited**

**U.S. PATENT DOCUMENTS**

4,093,474 6/1978 Sperry et al. ..... 148/11.5 A

*Primary Examiner*—R. Dean

*Attorney, Agent, or Firm*—Bachman and LaPointe

[57] **ABSTRACT**

In order to improve the weldability of aluminum strip or sheet by spot welding and to promote the use of these materials, in particular in the bodywork of automobiles, the strip or sheet, after being hot and cold rolled to an intermediate thickness of 1.5 to 2.5 times the final gauge, is etched in an alkaline solution, then cold rolled to final gauge using cold rolling lubricant and finally, if desired, heat treated.

**12 Claims, No Drawings**

**PROCESS FOR MANUFACTURING ALUMINUM  
STRIP OR SHEET HAVING IMPROVED  
WELDABILITY**

**BACKGROUND OF THE INVENTION**

The present invention relates to a hot and cold rolling process for manufacturing aluminum strip or sheet characterized by improved weldability, in particular aluminum strip about 0.1 to 0.7 mm thick for use in motor car bodies.

The use of aluminum sheet for manufacturing car body parts such as doors, engine bonnets, boot lids and wings is well known. Because of planned measures to save energy, in particular in view of the existing laws in the United States of America, vehicles will have to be made lighter. The increased use of strong and readily formable aluminum alloys for car body parts is therefore strongly anticipated.

Spot welding is widely used for joining components in car manufacturing, the lifetime of the electrodes used for welding steel sheet being about 10,000-15,000 welds. The corresponding number of welds with aluminum sheet is at present around 100-150 welds. After 25 that, the copper electrodes have to be cleaned to remove the aluminum which has alloyed itself with the copper.

The reason for the greater degree of alloying between aluminum and copper than between copper and steel is, besides the physical and thermodynamic properties of copper and aluminum which cannot be changed, the relatively marked variation in contact resistance between the copper electrode and the aluminum sheet. This is due mainly to the thickness of the oxide layer and the composition of the surface layer. It is well known that the contact resistance of aluminum alloys has a great influence on the ease of spot welding, the main reason for irregularity in welding and the short life-times of the electrodes used with untreated aluminum sheet being the high and non-uniform contact resistance at the point of current transfer. These affect energy conversion in the secondary circuit and cause marked variation in the quality of the joint.

Surface treatments such as brushing, sand blasting, wet jetting and caustic etching of the aluminum before spot welding markedly reduce the contact resistance. However, in the case of aluminum sheet, the rolled surface, when subjected to those treatments, becomes very rough. This affects the uniformity of the surface and detracts from the appearance of the part after lacquering.

It is therefore the principal object of the present invention to develop a process for producing readily 55 formable aluminum strip and sheet characterized by superior spot welding properties and furthermore housing a surface which is suitable for shaping and lacquering.

**SUMMARY OF THE INVENTION**

The foregoing object is achieved by way of the present invention wherein, after the strip or sheet has been hot and cold rolled to an intermediate thickness of 1.5 to 2.5 times the final thickness, it is etched in an alkaline 65 solution and then cold rolled to its final gauge using cold rolling lubricant. The strip may then be finally heat treated if desired.

**DETAILED DESCRIPTION**

It was found, surprisingly, that a considerable improvement in spot welding properties could be 5 achieved by removing the surface layer which raises the contact resistance, when the material has reached an intermediate thickness of 1.5-2.5 times the final gauge. The subsequent cold rolling and heat treatment detract only insignificantly from this good spot weldability. Consequently it is possible by subsequent cold rolling, to obtain a surface which is suitable for shaping and lacquering. This route is also more economical than treating the surface of the finished strip, as the surface area is smaller at the intermediate stage.

In this connection the aluminum alloys of the following composition have been found to be particularly favorable:

|    |             |     |               |                   |
|----|-------------|-----|---------------|-------------------|
| 1. | 0.4 to 1.5% | Mg, | 0.3 to 1.5%   | Si                |
| 0  | 0 to 0.03%  | Cu, | 0 to 0.5%     | Fe                |
| 0  | 0 to 0.1%   | Mn, | rest aluminum |                   |
| 2. | 0.3 to 6%   | Mg, | 0 to 1%       | Mn                |
| 0  | 0 to 0.4%   | Si, | 0 to 0.4%     | Fe                |
| 0  | 0 to 0.2%   | Cu, | 0 to 0.5%     | Cr, rest aluminum |
| 3. | 1.0 to 5.0% | Cu, | 0.4 to 2.5%   | Mg                |
| 0  | 0 to 0.8%   | Si, | 0 to 0.7%     | Fe                |
| 0  | 0 to 1.5%   | Mn  |               |                   |

These are then hot and cold rolled, subjected to caustic etching, rolled to final gauge and heat treated.

For the etching of the aluminum an alkaline solution is suitable and a solution of caustic soda, polyphosphate, wetting agents and inhibitors is preferred.

Also within the scope of the present invention is the use of aluminum strip or sheet as spot welded parts or devices, in particular sheet for car bodies, such that the aluminum strip or sheet, after being hot and cold rolled to an intermediate thickness of ca. 1.5 to 2.5 times the final thickness, is etched in an alkaline solution and then cold rolled to the final gauge using cold rolling lubricant, and then, if desired, heat treated.

**EXAMPLES**

45 One strip each of the following materials

- (a) Pure aluminum (98.7%)
- (b) AlMgSi containing 0.4% Mg and 1.2% Si, and
- (c) AlMg3

was produced in the following forms:

- 50 1. Without intermediate caustic etching i.e. by the normal production route,
- 2. with intermediate caustic etching and subsequent rolling down to final gauge before heat treating.

The contact resistance values between the copper electrode and these sheet materials are listed in the following table:

| 60       | Alloy | Version | Contact Resistance          |                         |
|----------|-------|---------|-----------------------------|-------------------------|
|          |       |         | Cu/Al sheet ( $\mu\Omega$ ) | Scatter ( $\mu\Omega$ ) |
| Al 98.7  |       | 1       | 32                          | $\pm 10$                |
|          |       | 2       | 13.1                        | $\pm 3$                 |
| AlMg 0.4 |       | 1       | 15.1                        | $\pm 6.3$               |
|          |       | 2       | 4.3                         | $\pm 2.2$               |
| Si 1.2   |       | 1       | 290                         | $\pm 40$                |
|          |       | 2       | 30                          | $\pm 5$                 |
| AlMg 3   |       | 1       |                             |                         |
|          |       | 2       |                             |                         |
| soft     |       | 1       |                             |                         |
|          |       | 2       |                             |                         |

What is claimed is:

1. A process for manufacturing aluminum sheet or strip characterized by improved weldability comprising:

rolling said aluminum sheet or strip to an intermediate thickness of from about 1.5 to 2.5 times the final gauge;

etching said rolled sheet or strip in an alkaline solution; and

rolling said etched sheet or strip to final gauge.

2. A process according to claim 1 wherein said aluminum sheet or strip is hot and cold to said intermediate thickness.

3. A process according to claim 1 wherein said aluminum sheet or strip is rolled to final gauge using a rolling lubricant.

4. A process according to claim 11 wherein said aluminum sheet or strip is cold rolled to final gauge.

5. A process according to claim 11 wherein said aluminum sheet or strip is cold rolled to final gauge using a cold rolling lubricant.

6. A process according to claim 1 further including the steps of heat treating said aluminum sheet or strip after rolling to said final gauge.

7. A process according to claim 1 wherein said aluminum sheet or strip comprises an aluminum alloy consisting essentially of 0.4-1.5% magnesium, 0.3-1.5% silicon, 0-0.03% copper, 0-0.5% iron, 0-1.0% manganese, balance aluminum.

8. A process according to claim 1 wherein said aluminum sheet or strip comprises an aluminum alloy consisting essentially of 0.3-6% magnesium, 0-1.0% manganese, 0-0.4% silicon, 0-0.4% iron, 0-0.2% copper, 0-0.5% chromium, balance aluminum.

9. A process according to claim 1 wherein said aluminum sheet or strip comprises an aluminum alloy consisting essentially of 1.0-5.0% copper, 0.4-2.5% magnesium, 0-0.8% silicon, 0-0.7% iron, 0-1.5% manganese, balance aluminum.

10. A process according to claim 1 wherein the etching is carried out in an alkaline solution consisting of caustic soda, polyphosphate, wetting agents and inhibitors.

11. A process according to claim 1 further including the steps of welding said aluminum sheet or strip into automobile body sheet.

12. A process according to claim 11 wherein said aluminum sheet or strip is spot welded.

\* \* \* \* \*

UNITED STATES PATENT AND TRADEMARK OFFICE  
CERTIFICATE OF CORRECTION

PATENT NO. : 4,326,895

DATED : April 27, 1982

INVENTOR(S) : WERNER HORN and JÜRGEN HENNINGS

It is certified that error appears in the above-identified patent and that said Letters Patent are hereby corrected as shown below:

Column 1, line 48, change "contrast" to --contact--.

Column 1, lines 57-58, change "housing" to --having--.

Column 1, line 63, after "wherein" delete ",".

Column 3, line 12, claim 2, after "cold" insert --rolled--.

Column 3, line 17, claim 4, change "11" to --1--.

Column 3, line 19, claim 5, change "11" to --1--.

Signed and Sealed this

*Fifteenth* Day of *February* 1983

[SEAL]

Attest:

GERALD J. MOSSINGHOFF

*Attesting Officer*

*Commissioner of Patents and Trademarks*